

## UNITED STATES PATENT OFFICE

2,664,353

MASTER ALLOY COMPRISING ZIRCONIUM  
AND MAGNESIUM FOR USE IN MAKING  
MAGNESIUM-BASE ALLOYS CONTAINING  
ZIRCONIUMWilliam P. Saunders and Frederick P. Strieter,  
Midland, Mich., assignors to The Dow Chemical  
Company, Midland, Mich., a corporation of  
DelawareNo Drawing. Application December 8, 1951,  
Serial No. 260,776

6 Claims. (Cl. 75—135)

1

The invention relates to methods of making magnesium alloys containing zirconium. It more particularly concerns the production of a master alloy containing both magnesium and zirconium in more or less equal proportions which is suitable for use in the production of magnesium-base alloys containing zirconium.

The zirconium metal commercially available alloys with magnesium but slowly and to a limited extent and is not generally used in making magnesium-base alloys containing zirconium. Instead a master alloy of magnesium and zirconium is preferably formed by reacting the molten magnesium with zirconium tetrachloride. The zirconium tetrachloride becomes reduced by molten magnesium to metallic zirconium according to the reaction expressed in the following equation:



In carrying out this reaction, the zirconium tetrachloride is mixed with the molten magnesium preferably in admixture with an alkali or alkaline earth metal chloride as a flux so as to reduce the tendency for some of the zirconium tetrachloride to become lost as dust or sublimate during the reaction. Examples of mixtures of zirconium tetrachloride and flux heretofore proposed are: (1)  $\text{ZrCl}_4 + \text{KCl}$  in equal amounts; (2)  $\text{ZrCl}_4$  50 parts +  $\text{NaCl}$  25 parts +  $\text{KCl}$  25 parts. It has also been proposed to include  $\text{BaCl}_2$  in the foregoing mixtures. Limited amounts of  $\text{CaCl}_2$  and  $\text{MgCl}_2$  may also be present in these mixtures. By employing about  $1\frac{1}{2}$  as much zirconium tetrachloride as magnesium in the reduction, a so-called master alloy is obtained containing more or less equal amounts of zirconium and magnesium and some entrapped by-product magnesium chloride, the rest of the saline constituents being removable from the metallic reaction mass by decantation and squeezing the mass. The master alloy consists essentially of a matrix of a magnesium-zirconium alloy, which is magnesium more or less saturated with zirconium (i. e. containing up to about 0.5 per cent of Zr), throughout which matrix is dispersed particles of zirconium metal comprising about 50 per cent by weight of the mixture. The amount of by-product magnesium chloride entrapped in the master alloy after decantation and squeezing is about 5 to 7 per cent of the weight of the master alloy.

2

In forming magnesium-base alloys containing zirconium by adding the so-prepared master alloy to melts of magnesium, there is danger of the molten magnesium undergoing such alloying of being blown about due to the violence with which the master alloy may react with melts of molten magnesium. This violence of the reaction, we have found, appears to be due to the magnesium chloride which is entrained in the master alloy during manufacture. Our investigations have shown that some of the entrained magnesium chloride, present in the master alloy, absorbs an amount of moisture from the ambient atmosphere prior to use which is dangerous to bring into contact with melts of molten magnesium as in making magnesium-base alloys with the master alloy. Such absorbed moisture on being brought into contact with molten magnesium, as in the alloying operation, produces a violent explosive-like reaction which causes more or less of the molten magnesium to be spattered about in dangerous manner. A peculiarity of this phenomenon is that it may not occur with every piece of the master alloy nor until the master alloy is well submerged below the surface of the molten magnesium to which the alloy is added, thus accentuating the hazard of the alloying operation. The danger of explosive-like reactions is greater the longer the lapse of time following manufacture of the master alloy.

We have now discovered that the foregoing dangers of alloying the magnesium-zirconium master alloy with melts of magnesium may be completely overcome by subjecting the master alloy to a puddling operation with a molten saline washing flux comprising one or both of the alkali metal chlorides,  $\text{NaCl}$  and  $\text{KCl}$ . If desired, barium chloride may be included in the washing flux but not in excess of 80 per cent of the weight thereof, thereby increasing its specific gravity. In the puddling operation, both the contaminated master alloy to be treated and the washing flux are maintained at a temperature at which the magnesium alloy portion of the master alloy is molten as well as the flux constituents. On thus melting the master alloy along with the washing flux, and puddling these materials together, the flux entrained in the master alloy is released and absorbed by the washing flux forming a mixture of spent washing flux containing the magnesium

## 3

chloride released from the master alloy. A sufficient amount of washing flux is used so that the magnesium chloride concentration in the spent flux mixture, formed in the puddling operation, is below about 5 per cent by weight. The spent flux mixture resulting from the puddling operation is separated from the resulting treated master alloy as by decantation and squeezing. The master alloy so separated from the spent washing flux is cast in a suitable mold and thereafter may 10 be used in making magnesium-base alloys containing zirconium without danger of explosions or undesirable boiling, spattering, and the like.

The washing flux is preferably thinly fluid at operating temperature and the desired fluidity is 15 achieved by making the flux of two or more of the proper chlorides so that the melting point of the flux mixture is preferably below about 1350° F., although saline fluxes melting as low as 900° F. and as high as 1480° F. may be used that do not 20 contain significant amounts of a hygroscopic alkaline earth metal chloride exclusive of BaCl<sub>2</sub>.

Examples of suitable saline fluxes for use according to the invention are set forth in the following table in parts by weight together with 25 the approximate temperature at which the flux is liquid.

| Flux No. | Flux constituents |      |     | Temper-<br>ature at<br>which flux<br>is liquid,<br>°C. |
|----------|-------------------|------|-----|--------------------------------------------------------|
|          | BaCl <sub>2</sub> | NaCl | KCl |                                                        |
| 1.       |                   | 100  | 100 | 1,479                                                  |
| 2.       |                   | 50   | 50  | 1,423                                                  |
| 3.       |                   | 25   | 75  | <1,200                                                 |
| 4.       |                   | 44   | 56  | 1,235                                                  |
| 5.       |                   | 72   | 28  | 1,195                                                  |
| 6.       |                   | 50   | 50  | 1,409                                                  |
| 7.       |                   | 70   | 30  | <1,300                                                 |
| 8.       |                   | 64   | 35  | 1,209                                                  |
| 9.       |                   | 70   | 30  | 1,193                                                  |
| 10.      |                   | 17   | 83  | 1,206                                                  |
| 11.      |                   | 55   | 20  | 1,382                                                  |
| 12.      |                   |      |     | 1,006                                                  |

In washing the master alloy with the washing flux, the master alloy may be heated, as in an open melting pot, to a temperature above its melting point along with about an equal weight of washing flux. The washing flux melts and serves to protect the melt from attack by the air during the melting and washing operation. The molten washing flux and the molten master alloy are mixed together so as to permit the washing flux to absorb and dilute the salines entrapped in the master alloy as made and released on being melted. A few minutes of stirring of the molten washing flux and master alloy suffices. Thereafter, the mixture is left to settle whereby the spent washing flux rises to the top of the molten metal which collects at the bottom of the melting vessel. The spent flux is separated from the molten metal as by decantation. If desired, the washing operation may be repeated once or twice.

The following example is illustrative of the practice of the invention:

## Example

A conventional master alloy is formed by melting 19 pounds of magnesium, heating the molten metal to 1400° F., and mixing with the molten metal 85 pounds of a mixture of equal parts of ZrCl<sub>4</sub> and KCl. In the reaction which ensues the ZrCl<sub>4</sub> is reduced to metallic zirconium forming magnesium chloride as a by-product. Part of the zirconium so-produced alloys with the balance of the molten magnesium while the remain-

## 4

der of the zirconium becomes dispersed in the magnesium-zirconium solution along with about 7 per cent by weight of by-product MgCl<sub>2</sub> thus forming the conventional master alloy containing about equals weights of magnesium and zirconium. The conventional master alloy settles under the supernatant layer of molten KCl containing the balance of the by-product MgCl<sub>2</sub> which is not entrained in the master alloy. The settled conventional master alloy so or otherwise produced is subjected to washing according to the invention. The supernatant layer of molten KCl and MgCl<sub>2</sub> is skimmed off and about 2 pounds of the master alloy is withdrawn from the flux-free surface of the molten mass thereof by dipping with a ladle. The so-removed master alloy is added to and mixed with a molten washing flux consisting of a melt of 15 pounds of BaCl<sub>2</sub> and 15 pounds of KCl at 1400° F. The mixing is continued for 3 minutes. The resulting washed master alloy is separated from the spent washing flux and solidified in an iron mold. Analysis of the so-obtained master alloy shows that the entrained MgCl<sub>2</sub> content is reduced to below 0.5 per cent. The solidified master alloy is put into storage. After storage for 3 days the master alloy is added to a melt of a magnesium-base alloy consisting of 95 pounds of magnesium and 5 pounds of zinc, melted in an open melting pot, thereby forming a magnesium-base alloy containing about 5 per cent of zinc and about 0.5 per cent of zirconium. The alloying takes place without any violence of reaction and with an efficiency of about 50 per cent. In contrast, when a similar amount of the conventional unwashed master alloy, after 3 days of similar storage, is added to and mixed with the same magnesium-base alloy under the same conditions in a similar melting pot there ensues an explosive reaction 40 ejecting molten metal from the melting pot.

The term "magnesium-base alloy" as used herein includes magnesium and alloys thereof in which the magnesium content is at least 80 per cent by weight.

We claim:

1. The method of making a master alloy comprising more or less equal amounts of magnesium and zirconium for alloying with magnesium to make magnesium-base alloys containing zirconium and at least 80 per cent of magnesium which comprises reacting a saline flux mixture comprising alkali metal chloride and zirconium tetrachloride with an excess of magnesium at a temperature between 1300° and 1450° C. so as to reduce the zirconium tetrachloride to metallic zirconium and produce magnesium chloride as a by-product, said metallic zirconium becoming entrained in the said excess of magnesium as a master alloy, withdrawing at least a portion of the so-produced master alloy and mixing it with a saline washing flux comprising an alkali metal chloride selected from the group consisting of sodium chloride and potassium chloride at a temperature at which both the said washing flux and master alloy are molten so as to release the entrained magnesium chloride from the master alloy and absorb the released magnesium chloride in the said washing flux, and separating the so-treated master alloy from the resulting flux mixture.

2. The method according to claim 1 in which the saline washing flux contains barium chloride in amount not over 80 per cent of the washing flux.

3. The method according to claim 1 in which

the saline washing flux comprises sodium chloride.

4. The method according to claim 1 in which the saline washing flux comprises potassium chloride.

5. The method according to claim 1 in which the saline washing flux comprises sodium chloride and potassium chloride.

6. The method according to claim 1 in which the saline washing flux consists of sodium chloride, potassium chloride and barium chloride, the amount of barium chloride not exceeding 80 per cent by weight of the flux.

WILLIAM P. SAUNDERS.  
FREDERICK P. STRIETER.

6  
References Cited in the file of this patent

UNITED STATES PATENTS

| Number    | Name        | Date          |
|-----------|-------------|---------------|
| 2,497,530 | Ball et al. | Feb. 14, 1950 |
| 2,497,531 | Ball et al. | Feb. 14, 1950 |

FOREIGN PATENTS

| Number  | Country       | Date          |
|---------|---------------|---------------|
| 533,264 | Great Britain | Feb. 10, 1941 |
| 624,304 | Great Britain | June 4, 1949  |